

May 9, 1939.

H. H. BEENY

2,157,948

## HARDENING OF METAL SURFACES

Filed June 17, 1937



Fig. 1.



Fig. 2.

*Inventor:*  
HERBERT H. BEENY  
*By* Dike, Calver & Gray  
*Attorneys.*

## UNITED STATES PATENT OFFICE

2,157,948

## HARDENING OF METAL SURFACES

Herbert H. Beeny, Coventry, England, assignor  
to The Monarch Machine Tool Company, Sidney, Ohio

Application June 17, 1937, Serial No. 148,754  
In Great Britain April 16, 1937

4 Claims. (Cl. 148—21)

This invention relates to the treatment of ferrous surfaces such as are capable of being hardened by being locally heated by means of a burner to a high temperature and then immediately cooled. The flame is progressively applied to the surface at a predetermined rate, the arrangement being such that there is not sufficient time for the heat to be conducted away to the interior of the article before the surface of the latter is quenched.

The specification accompanying the co-pending patent application of myself and Arthur H. Lloyd, Serial No. 148,752 describes a particularly satisfactory burner and cooler for treating a ferrous (for example, a cast-iron) surface in this way, and also an improved form of burner.

It is now found that in treating the surface of a cast-iron V-rail in this way there is a tendency for cracks to form along the apex of the rail. This is probably due to the fact of the flames, acting on the flanks of the rail, heating the apex of the rail to too great an extent; this resulting in the apex of the rail being hardened to a greater depth than the flanks of the rail.

When a V-rail is to be used as an inverted-V-rail for supporting a machine-tool slide, it is unnecessary for its apex to be hardened as the load is taken by the flanks of the rail.

The present invention is concerned with the surface-hardening of the operative face of a V-rail, to be used for supporting a machine-tool slide or some other slide, by flame-heating the flanks of the rail and immediately thereafter cooling them, as specified above; and it involves means acting to prevent the apex of the rail from being hardened in this manner so that the hardened flanks of the rail will be separated from one another by a relatively soft surface along the apex of the rail. Preferably the said means includes a jet of water or other cooling medium arranged to impinge on the apex of the rail in the vicinity of where the flanks are being flame-heated, the said jet preferably being directed backwardly. Conveniently the cooling medium from this jet is delivered at a higher pressure than that from the main jets.

In the accompanying diagrammatic drawing:—

Figure 1 is a perspective view of an inverted V-rail, for a lathe-bed, in association with a surface-hardening apparatus in accordance with the invention; and

Figure 2 is a cross-section of the rail indicating the result of the surface-hardening.

The drawing shows an elongated burner 10 of the kind described in the specification above-

mentioned, the burner having limbs 11, 11 inclined to one another according to the inclination of the flanks 12, 12 of the V-rail. It is secured by means of the union 13 to the main fuel supply pipe 14. The latter passes through lugs 15, 15, which are bolted to one another at 16, of a tray 17 built up of halves. Cooling liquid is supplied under pressure by a pipe 18, which also passes through the tray 17, to a balance chamber 19 from which are two pairs of cooling pipes 20, 20 directing the cooling liquid on to the respective flanks of the rail in the manner described in the specification above-mentioned. Outlet pipes 21 from the balance chamber carry surplus liquid to the tray, whence it can exhaust by the outlet 22. In addition, the pipes 23 carry cooling liquid at a higher pressure to the burner for interiorly cooling the latter, the outlet pipes therefor being marked 24 and 25. The outlet pipe 24 exhausts where convenient, but the outlet pipe 25 is in this instance bent round as shown, the end 26 of the pipe lying substantially in the plane of the two fuel jets 27 and being directed rearwardly.

The pressure delivered from the nozzle end 26 of the pipe 25 is greater somewhat than that delivered from the nozzles of the main cooling pipes 20, and the pressure is regulated to be sufficient to cause a film of water to flow along the part of the apex of the rail in the vicinity of the flames on either side, thus preventing the apex from becoming heated by the combined flames. The result is that only the two flanks are hardened, as indicated at 28, 28 in Figure 2, and this is an arrangement which is perfectly satisfactory as it is only the two flanks which carry the load.

The controls for regulating the respective pressures of the cooling pipes 20 and 25, and the combustible mixture, are not here shown. It will be understood that the main supply pipes may be clamped to one another as desirable and supported, with the various control means, from any convenient support which is adjustable and capable of being fed to carry the burner and coolers along the rail at the predetermined rate.

In this way it is possible to harden the operative surface of a cast-iron inverted-V-rail for use in supporting a machine-tool slide in a very satisfactory manner.

What I claim as my invention and desire to secure by Letters Patent of the United States is:—

1. A method of surface-hardening only the inclined flanks of a ferrous inverted-V rail, to be used for supporting a slide, which involves flame-

heating the flanks of the rail while directing a jet of cooling medium on to the apex of the rail adjacent the flanks, and immediately cooling the flanks after they have been heated, whereby the 5 hardened flanks will be separated from one another by a relatively soft surface adjacent the apex of the rail.

2. A method of surface-hardening only the inclined flanks of a ferrous inverted-V rail, to be 10 used for supporting a slide, which involves flame-heating the flanks of the rail while directing a jet of cooling medium on to the apex of the rail adjacent the flanks in a direction rearwardly of the direction of flame travel, and immediately 15 cooling the flanks after they have been heated, whereby the hardened flanks will be separated from one another by a relatively soft surface adjacent the apex of the rail.

3. Apparatus for use in surface-hardening the 20 inclined flanks of a ferrous inverted V-rail, to be used for supporting a machine-tool slide, including flame jets for flame-heating the flanks to a high temperature, jets of cooling medium directed on to said flanks for immediately cooling the

flanks after they have been heated, and a higher pressure jet of cooling medium directed to the apex of the rail in the vicinity of where the flanks are being flame-heated, whereby the apex is protected from heat hardening during the heating 5 of the said flanks.

4. Apparatus for use in surface-hardening only the inclined flanks of a ferrous inverted-V rail, to be used for supporting a slide, and including 10 a burner with divergent limbs inclined according to the inclination of the flanks and adapted to heat said flanks, a cooling system associated therewith and adapted to supply a cooling medium to said flanks subsequent to their heating, and means for preventing the heat hardening of 15 the apex of said rail and comprising a jet of said cooling medium directed on to the apex of the rail in the vicinity of the point of contact between said flanks and a heating flame, whereby the apex of said rail is preserved in a substantially 20 unhardened condition during the hardening of said flanks.

HERBERT H. BEENY.